

## UNITED STATES PATENT OFFICE

2,454,822

## LUBRICANTS FOR TEXTILE MATERIALS

Abraham Moscowitz, New York, N. Y., assignor  
to L. Sonneborn Sons, Inc., a corporation of  
Delaware

No Drawing. Application November 21, 1946,  
Serial No. 711,475

6 Claims. (Cl. 252—8.7)

1

This invention relates to new and useful improvements in lubricants for textile materials.

In textile processing such as of wool, worsted, rayon, viscose or the like, the raw materials are converted to fibres, the fibres formed into threads, the threads woven into fabric and the woven fabric further processed and finally dyed.

In the processing of wool or worsted, or the like, the raw material such as raw wool is subjected in pickers to an "opening" operation, i. e., freeing of the fibres as much as possible with a minimum of breakage. Thereafter the fibres are carded, i. e., fully opened and subjected to a "roving" operation, i. e., the formation of a continuous form of fibre or roving prior to spinning. The roving is spun into threads and the threads woven into fabric, the woven fabric being then fulled and finally dyed. These operations, up to the fulling step, including a variety of intermediate steps not herein enumerated, require the presence of a lubricating agent. This agent is conventionally added in the pickers prior to carding and may be applied either straight or in the form of emulsions. The latter is the more common procedure; the emulsion usually contains about 25% of the composition and is conventionally applied as a spray. The wool is impregnated to retain about 5 to 10% of the composition. Normally the conditions of processing are such that the water of the applied emulsion largely evaporates by the time the impregnated material is spun, the material ordinarily reaching this stage with a desired water content which may range for example from 5 to 15%, the preferred water content being inter alia dependent upon the type of material processed. The fulling step as such involves a mechanical beating of the fabric in drip-wet condition in the presence of a fulling agent and serves to densify the material, giving it its character, construction and appearance. Fulling agents may be either of the acid or of the alkaline type. Alkaline fulling agents are the more common and usually comprise about 6 to 8% soap. Two to four percent of soda are also conventionally added as an aid to the action of the fulling agent. The drip-wetness of the fabric in the fulling step is usually defined by a water content of between 80 and 100% and sometimes higher of water per dry weight of goods.

In conventional practices the lubricant on the fibre, such as wool, when reaching the fulling step is antagonistic to the fulling operation and largely prevents the necessary wetting contact of the water with the fibre. It is inter alia for this reason that such relatively large amounts of fulling agents have to be added, i. e., to counteract this action of the lubricant.

In the processing of synthetic materials such as rayon, viscose or the like, filaments as they come from the spinning solution or bath are converted into yarn and the yarn knitted or woven

2

into fabric. The formation of the yarn prior to the weaving includes such processing steps as carding, quilling and combing, all of which, together with the subsequent weaving or knitting, also necessitate the use of a suitable lubricant. Such lubricant is conventionally the same composition or of the same type as that used in wool processing and is normally applied to the loosely held together filament cakes either as such, i. e., straight, or in the form of aqueous emulsions. When the textile lubricant composition is applied by way of emulsion, usually a 1 to 4% aqueous emulsion is employed and penetrates the filament cake leaving on the fibre approximately 1/2 to 2% of the lubricant which in the majority of cases is satisfactory for the intended purpose. The lubricant at the same time acts as a softening agent. Once the filaments are converted into yarn, the yarn is first used for the setting of warp threads as the first step in the weaving operation. These warp threads are then first sized with a suitable size solution, such as gelatin or the like, to condition them for the subsequent weaving operation. Conventional textile lubricant impregnants are antagonistic to the size solution and it is necessary to incorporate a wetting agent in the size to overcome the repelling effect of the impregnant.

The hitherto used textile lubricants are also antagonistic to the dyeing operation of both wool type and synthetic type fibres in that they interfere with the requisite wetting contact between the dye bath and the fibre and must be removed therefore prior to the dyeing step. This removal is carried out in a scouring operation in which the goods are exhaustively washed with water containing scouring agents, such as soaps, usually in the presence of alkalis, such as soda ash. The use of the scouring agents, however, does not effectuate the substantially complete removal of the conventional lubricating compositions from the fibres of the fabric treated. Substantial complete removal of lubricant as generally understood in the art is defined as 85-90% or better removal (plant run test) of the lubricant used. In the majority of cases scourability of lubricating agents used in conventional practices normally results in lubricant removal of not better than about 65-77% by plant run test which is equivalent to about 60 to 70% by laboratory test, i. e., as determined by conventional laboratory scourability tests. (Plant run scourability values are usually about 10% higher than the values indicated by laboratory scourability tests.) By reason therefore of this insufficient scourability of the conventional impregnants appreciable amounts of lubricant are carried over into the dyeing bath and there necessitate the use of dyeing assistants. The use of soaps and/or alkalis in scouring operations often exercises a detrimental effect upon the fibres and/or fabric.

subjected to the scouring treatment. Further the necessity for the use of soaps and/or alkali in scouring operations requires considerable amounts of hot water to remove the scouring agents, which per se have a deleterious effect upon the dyeing operation or the shades and tints of the dyed fabric. All these factors contribute to render textile processing in the conventional manner a relatively costly and uneconomical operation.

One object of the invention comprises inter alia a lubricant for textile materials substantially free from the aforementioned defects inherent in conventional textile treating compositions, and which, when carried as impregnant on a textile material substantially eliminates the aforesaid drawbacks and disadvantages of conventional practices or products in the processing of textile materials.

The foregoing and further objects of the invention will be apparent from the following description.

When treating a petroleum distillate stock with fuming sulfuric acid under sulfonating conditions of acid amount and temperature in accordance with conventional refining practice, an oil layer and acid sludge layer are formed. The oil layer contains dissolved therein petroleum sulfonic acids, collectively referred to as mahogany petroleum sulfonic acids, which are recovered therefrom in accordance with conventional methods in the form of solutions of these sulfonic acids or their salts (herein collectively termed "petroleum mahogany sulfonates") in a portion of the oil relatively tenaciously occluded by these sulfonic bodies and generally referred to in the art as "retained oil." These petroleum sulfonic acids or sulfonate oil compositions normally contain about 30 to 35% of retained oil and 65 to 70% of the petroleum mahogany sulfonic material. Depending upon the type and origin of petroleum oil distillates from which these sulfonate-oil solutions or stocks are derived they contain sulfonates of varying averaged molecular weights. For convenience therefore the sulfonate stocks are identified by their averaged molecular weights. Thus a 420 or 450 sulfonate stock is a stock in which the sulfonates have an average molecular weight of 420 or 450 respectively.

Petroleum mahogany sulfonate solutions are extremely viscous in character even when reduced by the addition of further amounts of oil to as low as 20% sulfonate content, and are, as such, unsuitable for use as textile lubricants since it is a prerequisite for textile lubrication that the impregnating material does not normally exceed a viscosity of 600 seconds Saybolt at 100° F. This is by reason of the fact that higher than 600 seconds Saybolt viscosities will not flow sufficiently freely for satisfactory impregnation and will tend to such relative stickiness as to seriously impair their lubricating properties. Thinning with non-lubricating solvents is normally not successful as these will either evaporate, thus leaving behind a viscous, sticky impregnating material without adequate lubricating capacity on the fibre, or will interfere with the scouring operation. On the other hand, thinning with a textile lubricant type diluent will not obtain the desired result, as it is necessary to add so much of the diluent as to bring the sulfonate content to below that necessary for adequate emulsification or even minimum conventional scourability. Even disregarding the viscosity limitation the highest heretofore proposed amounts of 25% sulfonate content (Red-

dish U. S. 1,909,721, Twitchell U. S. 1,794,342) fail to impart substantial self-scourability.

In accordance with the invention the normally high viscosity of an alkali metal petroleum mahogany sulfonate solution in a textile lubricant hydrocarbon can be reduced to a point permitting the obtaining of such solution with a viscosity not exceeding 600 seconds Saybolt at 100° F. and containing in excess of 28% sulfonates, and 10 the impregnation of a textile material, prior to spinning or other fabrication into yarn, with lubricating amounts of such viscosity-reduced solution yields a substantially self-scouring lubricated textile product ready for further processing. 15 If the impregnated textile material is wool a substantially self-fulling as well as self-scouring lubricated wool is obtained. This impregnated wool permits a simplified processing in which it is subjected to a fulling operation with water in substantially drip-wet amounts and substantially free from fulling agents. The process may additionally include, after fulling, a scouring operation with substantially exhaustive amounts of water substantially free from scouring agents followed by dyeing, or, a dyeing operation without 25 prior scouring, i. e., with the impregnant substantially remaining in or on the wool when the same enters the dye bath. Thus in the case of wool the lubricating impregnant is per se fulling agent and also a dyeing assistant.

The aforementioned viscosity reduction is preferably carried out by subjecting the petroleum mahogany sulfonate textile lubricant hydrocarbon solution, containing in excess of 28% sulfonate and having by reason of the sulfonate content a viscosity in excess of 600 seconds Saybolt at 100° F., to a viscosity reducing reaction. The viscosity reducing reaction may be an oxidation reaction, i. e., a reaction in which an oxidation potential exists. The oxidation reaction may be induced by materials in which the oxidation potential exists by virtue of the presence or liberation of O<sub>2</sub>, such materials including inorganic oxidation agents such as chromic acid, bichromates, peroxides, etc., as well as organic oxidation agents and particularly organic peroxides such as benzoylperoxide, butylperoxide and similar materials. The oxidation reaction may be induced by materials in which the oxidation potential exists by reason of the presence of what is conventionally termed "active chlorine" as it is present in oxidatively acting chlorine, chlorine oxides, such as Cl<sub>2</sub>O and ClO<sub>2</sub>, or oxidatively acting derivatives, both inorganic and organic, 35 of the various chlorine-oxygen acids or their salts as for example hypochlorous acid (HOCl), hypochlorites, organic hypochlorous derivatives including those of the chloramine type such as toluene sulfonchloramide and benzene sulfon-chloramide, chlorous acid (HClO<sub>2</sub>), chlorites, as well as combinations of these "active chlorine" containing agents. Alternatively, the viscosity reducing reaction may be obtained by treatment with relatively small amounts of such agents as 40 various diethylene glycol esters and phthalic acid esters and particularly dimethyl phthalate.

The reaction conditions under which the oxidizing substances produce an oxidation potential are well known in the art and need not be further exemplified here except with respect to the preferred procedures for the procurement of maximum chlorine oxidation potentials herein-after noted.

Particularly good results are obtained by carrying out the chlorine oxidation reaction with

a hypochlorite at a pH range of about 6-8 and preferably at a neutral to alkaline pH, or, with alkali metal chlorite at an acid pH. Thus for instance the hydrocarbon solvent solution of a suitable mahogany sulfonate may be subjected to a hypochlorite treatment substantially as set forth in the Blumer et al U. S. Pat. 2,201,119 using amounts of hypochlorite sufficient to obtain the desired viscosity reduction which is accompanied by the color reduction to a Lovibond value of less than 8R (10% white oil solution  $\frac{1}{2}$ " cell) as set forth in said patent. Alternatively, such solution may be intimately contacted with a suitable chlorite at a pH below 7 in accordance with the procedure set forth in the Liberthson et al. patent, U. S. 2,307,743, using amounts of chlorite sufficient to obtain the desired viscosity reduction which is accompanied by the color reduction to a Lovibond value of less than 8R (10% white oil solution  $\frac{1}{2}$ " cell) as set forth in said patent.

For best results, however, a combination of the chlorite and hypochlorite treatment is preferred. In the preferred mode of such treatment, 1.5-7% and preferably 2.5-6% of the chlorite and hypochlorite (calculated in the aggregate dry weight by weight of sulfonate in solution) are used in a proportion of 0.5 to 4 parts by weight and preferably of 2 to 3 parts by weight of hypochlorite for every one part by weight of chlorite. The viscosity reduction reaction is carried out with this procedure by intimately contacting the chlorite hypochlorite combination with the sulfonate hydrocarbon solution until the desired viscosity reduction is obtained. The pH of reaction may be on the alkaline or acid side avoiding an excess on either side. When operating on the acid side neutralization is necessary. This is usually accompanied by some increase in viscosity of the reaction reduced viscosity. For this reason it is of advantage to select the pH of reaction at 7 or higher and preferably at from 7.5-8.5; if necessary the solution may be acidified with  $H_2SO_4$  to that range. The preferred mode of operation is to dissolve the chlorite in the aqueous hypochlorite solution. The temperature is ordinarily not critical. The reaction however may be facilitated by increasing the temperature to for example a preferred temperature of from 120° to 200° F.; this will increase the fluidity of the petroleum hydrocarbon, thus permitting more intimate contact between the reactants. The combination chlorite-hypochlorite treatment within the preferred scope of my invention effectuates a larger viscosity reduction with a lesser amount of total chlorine oxidation reagents than is the case with either the chlorite or hypochlorite treatment alone.

The viscosity reducing reaction is carried out as stated on a textile lubricant hydrocarbon solution of in excess of 28% alkali metal petroleum mahogany sulfonate content, which solution possesses normally a viscosity in excess of 600 seconds Saybolt at 100° F. due to the sulfonate dissolved therein. The petroleum mahogany sulfonate content may be so selected that after the completion of the viscosity reducing reaction the resulting product is per se usable, after such further refining or purification (including removal of inorganic salts, if necessary) as may be required, as a textile treating oil, i. e., possessing a viscosity below 600 and a petroleum mahogany sulfonate content in excess of 28% and preferably between 28 and 40%. Alternatively, the viscosity reducing reaction may be carried out with

a textile lubricant hydrocarbon solution containing relatively high concentrations of petroleum mahogany sulfonate, as for instance in excess of 40% petroleum mahogany sulfonate, in which case the resultant product is a concentrate which must then be adjusted by the addition of textile lubricant hydrocarbon of suitable viscosity to the requisite petroleum mahogany sulfonate content, i. e., in excess of 28% and preferably between 28 and 40% and a viscosity below 600 and preferably for wool below 500 and for synthetic fibre below 300 seconds Saybolt at 100° F. Generally solvent extension to reduce viscosity of a treated concentrate to below 600 seconds Saybolt at 100° F. will simultaneously bring the sulfonate content to 40% or lower. The viscosity of the extending hydrocarbon lubricant should be so selected that the viscosity of the finished product is maintained below its desired top limit. In the viscosity reducing reaction, inorganic salts are formed which if produced in excessive amounts may sufficiently interfere with the emulsifying or wetting or re-wetting properties of the resultant product to make their removal in the conventional manner advisable. In many cases however such relatively small quantities of inorganic salts are formed as are insufficiently large to materially impair the desirable textile processing properties of the impregnant. These can then be carried into the finished product without necessity for removal.

When proceeding in accordance with the invention it is in most cases of advantage to use the sulfonate product obtained in the conventional acid refining petroleum oil distillates and containing about 61-2% petroleum mahogany sulfonates (having an average molecular weight for example of from 400-550) and about 37-8% "retained" oil. Such a product may normally possess, for instance, a viscosity of about 80 to 205 furol at 210° F. and, after treatment with, for instance, the chlorite hypochlorite combination, a reduced viscosity of between 38 and 112 furol at 210° F. which when diluted with a hydrocarbon and preferably a mineral oil stock of suitable viscosity such as 75 seconds Saybolt at 100° F. to a 30% sulfonate content yields a viscosity of about 370 to 380 seconds Saybolt at 100° F.

Alternatively, the novel impregnant may be obtained directly as such, i. e., without necessity for adjustment with extending amounts of hydrocarbon oil, by a modification of the conventional acid refining procedure. When proceeding in this manner a petroleum oil distillate (containing about 30-35% sulfonates) is given at a temperature of about 150° F. a 50% batch treatment with fuming sulfuric acid, i. e., a treatment (sometimes in several batches) with 50% of acid by weight of the oil treated. The cooled acidified oil is thereafter diluted with an equal volume of benzol, the mixture is permitted to settle overnight and the acid sludge layer is withdrawn. After neutralizing the oil layer and removing the benzol by distillation, the oil layer is subjected to a suitable viscosity reducing reaction in accordance with the invention and preferably any of the herein described chlorine oxidation reactions. The resulting products contain approximately 70% of textile lubricant mineral oil and 30% of petroleum mahogany sulfonates and substantially possess a viscosity below 600 seconds Saybolt at 100° F.

The expression "textile lubricant hydrocarbon" or such similar term as used herein is intended to

designate a hydrocarbon or a hydrocarbon mixture such as a mineral oil or petroleum hydrocarbon oil, as it is conventionally used for textile lubricating purposes and having normally a minimum viscosity of about 40-50 seconds Saybolt at 100° F.; the maximum viscosity of the hydrocarbon or hydrocarbon mixture is limited in accordance with the invention so as not to bring the viscosity of the final composition above 600 and preferably 300 seconds Saybolt at 100° F. and in most cases the practical upper viscosity for the lubricant hydrocarbon within the 600 seconds limit is about "150 seconds" Saybolt at 100° F. and within the "300 seconds" limit about 65 seconds Saybolt at 100° F.

Wherever reference is made herein to the expression "lubricating amounts" in connection with my new lubricating impregnant on a textile material in accordance with the invention or where such similar term is used it is intended to designate thereby the amount of lubricant conventionally carried or required to be carried by a textile material for adequate lubrication in the processing thereof and which, for example, in the case of wool, worsted or similar materials may average about 2 to 10% lubricant on the fibre and in the case of a synthetic material such as viscose, rayon or the like may average about 0.25 to 2% lubricant on the fibre.

The novel lubricant composition when carried by the material, promotes rather than repels the contact-wetting of the fibre with water. For this reason, therewith impregnated wool is essentially self-fulling while a therewith impregnated synthetic fibre is essentially self-wetting with respect to a size solution.

In wool fulling it is desirable for best results to operate at a slightly alkaline pH and to this end small amounts of soda, up to for example 2% (by weight of the fulling water) may be added to further facilitate the fulling action of the impregnant. Other than this, however, no soap and no amounts in excess of 2% of soda ash are required.

The composition carried by the fabric in accordance with the invention not only acts as a fulling agent but continues during the fulling operation its lubricating function, thus resulting in more efficient fulling and production of an improved material. In effect therefore the instant invention permits the functional carrying of the lubricant from the dry part of the wool processing into the wet part of the wool processing operation. In the case of conventional wool lubricants, the lubricant function of the material ceases at the end of the dry part of the procedure and is carried over into the wet part without substantially there exercising any beneficial function, being in fact detrimental to the wet-precessing steps.

Thus, as above pointed out, when proceeding in accordance with the invention as applied to wool there is obtained a lubricant impregnated wool at the beginning of the textile processing operation, in which the impregnant as such is an efficient lubricating and fulling agent, eliminating the necessity for the otherwise costly and cumbersome conventional steps of adding a fulling agent in the fulling operation and a scouring agent in the scouring operation. The lubricant impregnated wool fabric in accordance with the invention emerges from the water scour with at least 90% (plant run test) of the impregnating agent removed. The lubricant on the wool constitutes in itself a dyeing aid and permits the

direct dyeing of the wool, after fulling, without a prior scour. In the latter case, it is recommended, however, that the impregnated material be given a light rinse after fulling, so as to substantially remove any pH controlling agents, as for example small amounts of soda ash, that may have been used in the fulling and which may be harmful to the dyeing or the shades of the dyed material. Some of the lubricant is removed with the rinse. All lubricant on the fibre when it enters the dye bath is effectively removed by the aqueous dyeing medium during the dyeing operation. The novel lubricant actually improves the dyeing characteristics of wool impregnated therewith and is not a deterrent to satisfactory dyeing, such as are conventional type compositions. By this procedure of using the lubricant composition in accordance with the invention as a fulling aid, a "hand" of material far superior to that obtained from products processed in the conventional manner is obtained.

My novel lubricant impregnant as it is present on the fibre and containing in excess of 28% sulfonate is substantially spontaneously dispersed, when contacted by water, in a manner assuring such fineness of dispersed globules of lubricant in the water of contact that the dispersion is of a magnitude approaching true solution, i. e., the majority of the dispersed globules are in the average of a magnitude of size below that of the average wave length of normal light, resulting in the formation of dispersions that are substantially translucent and for practical purposes transparent, and thus essentially approach true solutions. Thus the lubricant impregnants used in accordance with the invention are not only highly wettable, i. e., emulsifiable ab initio, but are also truly rewettable or reversible, after application to the fibre. They are substantially unaffected by any surface activity of or within the fibre and are substantially to the same extent remulsifiable upon water contact as they originally were when not on the fibre. In the fulling operation of for example wool, at least part of the novel impregnant is emulsified. Since only drip-wet amounts of water are used however in fulling, the impregnant is substantially retained in or on the wool during the physical working of the fulling operation. At the same time the pH controlling agent, preferably used when fulling in accordance with the invention, as for example soda, exercises a somewhat deterrent effect upon the emulsification of the impregnant and reduces the capacity of the fulling water for the amount of impregnant which it is able to emulsify. Ordinary viscosity unreduced textile lubricant hydrocarbon impregnant compositions, are restricted to a maximum of about 15-20% sulfonate content in order not to exceed the maximum usable viscosity limit and do not so react when on the fibre. These, and even compositions containing as high as 25% sulfonates, when contacted by water, produce ordinary opaque, milky-emulsion type dispersions, in which the particle size of dispersed globules is in the average above that of the average wave length of normal light. The surface activity of the fibre brings then into play forces of differential adsorption with respect to these type globules resulting in a relatively tenacious retention of at least a portion of the lubricant composition. This is one factor in the unsatisfactory scourability of a textile material impregnated with a conventional type mineral oil composition.

The following examples are furnished by way of illustration and not of limitation:

*Example I*

100 lbs. of a 450 petroleum mahogany sulfonate stock containing 61-2% mahogany sulfonates and 37-38% retained oil was used. The stock was obtained from a Mid-Continent stock subjected to white oil refining with fuming sulfuric acid under sulfonating conditions. 10 lbs. of an approximately 10% aqueous sodium hypochlorite solution (about 10% available Cl) were added to the mahogany sulfonate stock and the mixture was thereupon agitated, being kept at a temperature of between 200 and 220° F. The pH of the stock after addition of the hypochlorite was adjusted to pH 7 by the addition of small amounts of concentrated sulfuric acid. Agitation and heating were continued until samples drawn at frequent intervals indicated a Lovibond color reduction to about 2-3R (10% white oil solution  $\frac{1}{2}$ " cell). The desired result was achieved after about one-half hour. The major portion of the water added with the aqueous hypochlorite solution evaporated during the treatment. Before treatment the petroleum sulfonate stock had a viscosity of 144 furol at 210° F. and upon dilution with a mineral pale oil (75 seconds Saybolt at 100° F.) to a 30% sulfonate content, a viscosity of 1100 seconds Saybolt at 100° F. After treatment and before dilution the corresponding viscosity was 74 furol at 210° F. and after dilution with the same 75 viscosity pale oil, 395 seconds Saybolt at 100° F.

*Example II*

100 lbs. of the same 450 petroleum mahogany sulfonate stock as specified in Example I was adjusted to a pH of 6 to 6.5 and then about 3 lbs. of sodium chlorite was added in the form of a concentrated aqueous solution. The mix was agitated, maintaining the temperature at about between 180 and 200° F. Samples were taken at frequent intervals and the treatment discontinued when a color reduction to about 2-3R (Lovibond 10% white oil solution  $\frac{1}{2}$ " cell) was observed. This result was achieved after about one-half hour. After treatment the reduced viscosity was 72 furol at 210° F. and after dilution with the same 75 viscosity pale oil specified in Example I, 400 seconds Saybolt at 100° F.

*Example III*

100 lbs. of petroleum sulfonate-retained oil stock

containing 61-2% sodium sulfonates) were heated to 120° F.; a solution of 1 lb. sodium chlorite in 5 lbs. aqueous hypochlorite solution having a 10% available chlorine content was added. The mixture was heated to 200° F. and maintained at this temperature, while stirring, for one-half hour, then blown with air to drive out retained moisture and diluted with 75 viscosity mineral oil to a 30% sulfonate content. Before treatment, the petroleum sulfonate-retained oil stock had a viscosity of 163 furol at 210° F. and upon dilution to 30% sulfonate content 1463 Saybolt at 100. After treatment and before dilution the corresponding viscosity was 113 furol at 210 and after dilution 375 Saybolt at 100° F.

*Example IV*

100 lbs. of a stock as used in the preceding Examples I, II or III was diluted with a 70 viscosity (seconds Saybolt at 100° F.) mineral white oil to obtain a 30% mahogany sulfonate petroleum hydrocarbon solution. To this was then added 1 lb. of sodium chlorite dissolved in 2½ lbs. of an aqueous sodium hypochlorite solution (about 10% available Cl content). The mix was agitated and the temperature maintained at about 180 to 200° F. The pH was adjusted to about 8. The treatment was discontinued after a sample showed a reduced Lovibond color of about 2-3R (10% white oil  $\frac{1}{2}$ " cell). This result was achieved after about one-half hour. The solution before treatment possessed a viscosity of about 920 seconds Saybolt at 100° F. and after treatment with the chlorite-hypochlorite combination, a reduced viscosity of about 395 seconds Saybolt at 100° F.

In the following table comparative viscosity data are furnished of various sulfonate stocks showing in each case the viscosities of the untreated stock and of dilutions thereof to 30, 35 and 40% sulfonate content, respectively, as against the viscosities of the same stock, treated with hypochlorite, chlorite or the chlorite-hypochlorite combination, respectively, and of 30, 35 and 40% sulfonate dilutions for each treated stock. The respective treatments were carried out as specified in Examples I, II or III. The extending oil in each case was a neutral solvent refined mineral pale oil having a Saybolt viscosity of 75 or 50 seconds at 100° F. as specified.

| Type of Sulfonate Stock |                 | Percent Sodium Sulfonate | Furol Vis. at 210° F. | Saybolt Viscosities at 100° F. When Extended With 75 vis. neutral to Sodium Sulfonate Content |       |       | Viscosity Reductions Obtained By Treatments as Shown |                       |     |                              |     |                       |     |     |     |  |
|-------------------------|-----------------|--------------------------|-----------------------|-----------------------------------------------------------------------------------------------|-------|-------|------------------------------------------------------|-----------------------|-----|------------------------------|-----|-----------------------|-----|-----|-----|--|
|                         |                 |                          |                       | 30%                                                                                           | 35%   | 40%   | Na Hypochlorite alone in alk ph                      |                       |     | Na Chlorite alone in acid ph |     |                       |     |     |     |  |
| Av. Mol. Wt.            | Source          |                          |                       | Furol Vis. at 210° F.                                                                         | 30%   | 35%   | 40%                                                  | Furol Vis. at 210° F. | 30% | 35%                          | 40% | Furol Vis. at 210° F. | 30% | 35% | 40% |  |
| 500.....                | Gulf Coast..... | 62                       | 205                   | 1,500                                                                                         | 1,750 | 2,100 | 112                                                  | 470                   | 545 | 590                          | 108 | 475                   | 545 | 590 |     |  |
| 450.....                | Mid. Cont.....  | 62                       | 144                   | 1,100                                                                                         | 1,280 | 1,475 | 74                                                   | 395                   | 490 | 570                          | 72  | 400                   | 492 | 576 |     |  |
| 420.....                | Penna.....      | 62                       | 81                    | 910                                                                                           | 1,050 | 1,200 | 38                                                   | 375                   | 470 | 560                          | 40  | 375                   | 472 | 562 |     |  |

| Type of Sulfonate Stock |                 | Combination Chlorite-hypochlorite |                                                                                               |     |     |                                                                                               |       |       |       |       |       |
|-------------------------|-----------------|-----------------------------------|-----------------------------------------------------------------------------------------------|-----|-----|-----------------------------------------------------------------------------------------------|-------|-------|-------|-------|-------|
|                         |                 | Furol Vis. at 210° F.             | Saybolt Viscosities at 100° F. When Extended With 75 vis. neutral to Sodium Sulfonate Content |     |     | Saybolt Viscosities at 100° F. When Extended With 50 vis. neutral to Sodium Sulfonate Content |       |       | 30%   | 35%   | 40%   |
| Av. Mol. Wt.            | Source          |                                   | 30%                                                                                           | 35% | 40% | 30%                                                                                           | 35%   | 40%   |       |       |       |
| 500.....                | Gulf Coast..... | 110                               | 475                                                                                           | 550 | 590 | -----                                                                                         | ----- | ----- | ----- | ----- | ----- |
| 450.....                | Mid. Cont.....  | 73                                | 400                                                                                           | 495 | 575 | -----                                                                                         | ----- | ----- | ----- | ----- | ----- |
| 420.....                | Penna.....      | 39                                | 380                                                                                           | 475 | 560 | 185                                                                                           | 240   | 285   | ----- | ----- | ----- |

## 11

The following examples show various illustrations of the processing of textile materials in accordance with the invention.

## Example V

820 lbs. of tailors' clips were impregnated with a solution of 75 lbs. of a 30% petroleum sulfonate-mineral oil blend (prepared in accordance with the procedure described in Examples I, II, III or IV) in 300 lbs. of water heated to 160° F. The impregnation was accomplished by spraying the solution on the clips at the rate of about 4 gals. per 100 lbs. of clips. The impregnated clips were allowed to remain overnight to insure complete saturation and then run through a picker. The picked stock was then blended with 18% cotton and again the blend run through a mixing picker. The blend was then carded (there was no gumming on the cards) and spun into yarn. The yarn was then woven into fabric with cotton as the warp. The fabric was fulled without soap in water rendered slightly alkaline with about 2 oz. of soda ash per gallon of water. After fulling, the fabric was scoured at 100° F. for about one-half hour with plain water. There was copious sudsing and every indication of good detergency and dirt dispersion. Following the scouring, the fabric was rinsed and dyed in the normal manner, no assistant being added to the dye bath. The final fabric was superior in hand and general appearance to the normal mill run in which in the scouring operation 4 oz. soda ash and 6 oz. soap per gallon were used, and with the scouring of which additionally equal quantities of alkali and soap were required.

## Example VI

75 denier acetate yarn was impregnated with the solution of petroleum sulfonates used in Example V at 120° F. and scoured out at 140° F. with plain water. Analysis for matter extractible with ether showed 90.2% scourability. Similar runs with 25% solution of petroleum sulfonates in oil gave a scourability of only 68.5% and after using soap and soda ash in amounts given in Example V as scouring assistants, a scourability of 77% was determined.

## Example VII

A 25% emulsion of a 30% viscosity reduced mahogany sulfonate solution, as is obtained for instance in accordance with Examples I, II, III or IV, was prepared. This emulsion was then applied at a temperature of about 130° F. to wool stock in the picker at a rate leaving on the wool about 24% (by weight of the wool) of the emulsion, i. e., an equivalent of about 6% of the sulfonate impregnant. The emulsion was used in the form of a spray. The impregnated wool was then carded, spun to yarn and woven into fabric. Prior to subjecting the fabric to a fulling operation, the same was soaked to drip-wetness with water containing about 2% of soda ash and in this drip-wet condition was then subjected to fulling in the usual manner. Upon leaving the fulling mill, the fulled fabric was subjected to a scouring operation by repeatedly washing the same with plain water (i. e., without addition of scouring agent) having a temperature of approximately 105 to 110° F. until substantially all of the impregnant and other impurities were removed. As compared with the amounts of scouring water required for wool goods carrying conventional impregnants, the fulled material obtained in this case required considerably less

## 12

scouring water and the time of scouring and rinsing treatment was reduced to about half of that normally required by goods impregnated with conventional type impregnants. After scouring, extraction tests showed removal of impregnant to an extent of about 96%.

## Example VIII

Wool goods impregnated and processed as described in Example VII and as they come from the fulling mill were subjected to a rinse in the dyeing machine with weakly ammoniacal water and after removal of the aqueous rinsing medium were dyed in the normal manner. After dyeing extraction tests showed removal of impregnant in the dye bath to an extent of 95%.

## Example IX

A 1% aqueous emulsion was prepared using a 30% viscosity reduced (185 seconds Saybolt at 100° F.) mahogany sulfonate lubricant solution as for instance obtained by subjecting a 420 Pennsylvania sulfonate stock to the procedures set forth in Examples I, II or III and extending with a 50 vis. neutral (see table, last column). Viscose filament cakes were contacted with this emulsion for a time sufficient to leave on or in the filaments, after removal of excess emulsion, about  $\frac{1}{2}$  to  $\frac{3}{4}$  % (by dry weight of the filament) of the sulfonate lubricant. The emulsion soaked filament cakes were then centrifuged for removal of excess emulsion and the filaments dried and coned. The coned filaments were then "warped" and thereafter sized with the application of a size solution containing about 4% gelatin but no wetting agent. After treatment, about 2% of size is left on the warp whereupon the goods were woven into fabric and the fabric subjected to a boil-off operation by immersing the same in weakly ammoniacal hot water of about 140 to 150° F. No scouring or boil-off agent was used in the boil-off. The goods were then subjected to a dyeing operation in the usual manner. The goods exhibited level dyeing. Extraction tests of the boiled off goods showed removal of impregnant to an extent of about 95%.

The percentage impregnant removed on scouring or boil-off shown in Examples V-IX was ascertained in the usual manner by soxhlet ether extraction. The extracted material showed the residue left on the fibre after scouring or boil-off, thus indicating the amount of impregnant actually removed by that operation.

Instead of using for the wool or synthetic fibre impregnation as specified in Examples V to IX any of the viscosity reduced impregnants obtained in accordance with Examples I, II, III or IV, any other suitable viscosity reduced mahogany sulfonate hydrocarbon solution may be used as may be for instance obtained by other viscosity reducing treatment such as with  $\text{Cl}_2$ ,  $\text{ClO}_2$ , dimethyl phthalate or any other similarly reacting material.

The extent to which low viscosity values may be obtained depends, at least to some extent, upon the type or origin of the petroleum mahogany sulfonate selected for the treatment. Ordinarily high average molecular weight sulfonates possess a higher viscosity and the resulting viscosity after treatment is usually commensurately higher than the viscosity after treatment of a comparative sulfonate hydrocarbon solution which before treatment possessed a relatively lower viscosity and in which the sulfonate had a 75 lesser average molecular weight.

The foregoing description is for purposes of illustration and not of limitation and it is therefore my intention that the invention be limited only by the appended claims or their equivalents wherein I have endeavored to claim broadly all inherent novelty.

I claim:

1. A textile treating agent which comprises a hydrocarbon textile lubricating oil and substantially dissolved therein at least 28% alkali metal petroleum mahogany sulfonate obtained by reacting a petroleum mahogany sulfonate solution in an organic substantially water immiscible solvent for said sulfonate, with an oxidation agent selected from the group consisting of oxidation agents having an oxidation potential in such solution by reason of "available" O<sub>2</sub> and those having an oxidation potential in such solution by reason of "available" Cl<sub>2</sub> in amount and for a period of time sufficient to yield for its said at least 28% sulfonate solution a Saybolt viscosity at 100° F. of not in excess of 600 seconds.

2. A textile treating agent in accordance with claim 1 in which said hydrocarbon textile lubricating oil contains dissolved therein from 28 to 40% of the said oxidation agent reacted petroleum mahogany sulfonate.

3. A textile treating agent in accordance with claim 2 in which said alkali metal petroleum mahogany sulfonate is one obtained by reaction with said oxidation agent in amount and for a period of time sufficient to impart to its said hydrocarbon textile lubricating oil solution a Saybolt viscosity at 100° F. of not in excess of 300 seconds.

4. A textile treating agent which comprises a hydrocarbon textile lubricating oil and substantially dissolved therein from 28 to 40% alkali metal petroleum mahogany sulfonate obtained by reacting a petroleum mahogany sulfonate solution in an organic substantially water immiscible solvent for said sulfonate, with an oxidation agent having an oxidation potential in said solution by reason of "available" O<sub>2</sub> in amount and for a period of time sufficient to yield for its said at least 28 to 40% sulfonate solution a Saybolt viscosity at 100° F. of not in excess of 600 seconds.

5. A textile treating agent which comprises a hydrocarbon textile lubricating oil and substantially dissolve therein from 28 to 40% alkali metal petroleum mahogany sulfonate obtained by reacting a petroleum mahogany sulfonate solution in an organic substantially water immiscible solvent for said sulfonate, with an oxidation agent having an oxidation potential in said solution by reason of "available" Cl<sub>2</sub> in amount and for a period of time sufficient to yield for its said at least 28 to 40% sulfonate solution a Saybolt viscosity of 100° F. of not in excess of 600 seconds.

6. A substantially self-scouring lubricated textile material which comprises a textile material impregnated with a viscosity reduced petroleum mahogany sulfonate solution consisting of a hydrocarbon textile lubricating oil and substantially dissolved therein at least 28% alkali metal petroleum mahogany sulfonate obtained by reacting a petroleum mahogany sulfonate solution in an organic substantially water immiscible solvent for said sulfonate, with an oxidation agent selected from the group consisting of oxidation agents having an oxidation potential in such solution by reason of "available" O<sub>2</sub> and those having an oxidation potential in such solution by reason of "available" Cl<sub>2</sub> in amount and for a period of time sufficient to yield for its said at least 28% sulfonate solution a Saybolt viscosity at 100° F. of not in excess of 600 seconds.

ABRAHAM MOSCOWITZ.

#### REFERENCES CITED

35 The following references are of record in the file of this patent:

#### UNITED STATES PATENTS

|    | Number    | Name          | Date          |
|----|-----------|---------------|---------------|
| 40 | 1,909,721 | Reddish       | May 16, 1933  |
|    | 2,122,593 | Stafford      | July 5, 1938  |
|    | 2,151,711 | Moscowitz     | Mar. 28, 1939 |
|    | 2,201,119 | Blumer et al. | May 14, 1940  |
|    | 2,307,743 | Liberthson    | Jan. 12, 1943 |
|    | 2,388,677 | Cohen         | Nov. 13, 1945 |
| 45 | 2,396,673 | Blumer        | Mar. 19, 1946 |